# EUROPEAN PATENT APPLICATION

(11) **EP 1 094 148 A1**
(43) Date of publication of application: **25.04.2001**
(21) Application number: 00660129.8
(22) Date of filing: 20.07.2000
(51) Int. Cl.: D06P 5/15

(54) **Method for patterning a textile product**

(30) Priority: 22.10.1999 FI 992290
(71) Applicant: Ruppa, Raili, 40200 Jyväskylä (FI)
(72) Inventor: Ruppa, Raili, 40200 Jyväskylä (FI)
(74) Representative: Hakola, Unto Tapani

(57) **Abstract**

The invention relates to a method for patterning a textile product made at least partly of wool, animal hair, silk or polyamide, by means of discharge printing, in which method colour is removed from a dyed textile product or a textile product of natural colour to attain a desired pattern. The invention also relates to a discharging agent containing at least one oxidizing agent intended for decolourisation. Moreover, the invention relates to the use of products intended for decolourisation of hair for producing patterns by means of discharge printing on the surface of a textile product made at least partly of wool, animal hair, silk, or polyamide.

## Description

The present invention relates to a method for patterning a textile product made at least partly of wool, animal hair, silk or polyamide by means of discharge printing. By animal hair reference is made to animal hair used in textile products, such as mohair, cashmere, angora, as well as hair of rabbit, camel, llama, vicuna or alpaca. By textile product reference is, in this application, made to textile structures suitable as surfaces to be discharged printed, such as woven fabric, knitted fabric or felt cloth. The woven fabric may be for example upholstery fabric or clothing fabric. The textile product may be in the form of a finished product, as an example it is possible to mention for instance a carpet, a sweater or a silk scarf.

The patterning of a textile product can be conducted by means of methods related to weaving techniques, such as jacquard weaving, or by patterning a knitted fabric by means of jacquard and inlaid knitting, or by printing with textile dyes, or by discharge printing.

By means of discharge printing, the patterning is conducted in such a manner that colour is removed from a certain point of a dyed textile product or a textile product of natural colour to produce the patterning. The colour can be removed entirely or partly in such a manner that the desired hue is attained. The point from which colour has been removed can be left in the state in which it is after the decolourisation (resulting in white or pale colours, so called resist white) or the substance removing the colour, i.e. so called discharging agent is supplemented with another dye (resulting in coloured patterns, so-called coloured resists). The discharge printing enables the production of large patterns of free form.

Wool, animal hair and silk are protein fibres, in the dyeing and decolourisation of which it is possible to use similar kinds of substances. As for man-made fibres, polyamide has a chemical structure resembling the protein fibres with respect to dyeing and decolourisation, and therefore polyamide can also be treated with the method according to the invention. However, it is necessary to select suitable processing conditions and/or auxiliary substances for each fibre.

According to prior art, the decolourisation is conducted by means of a reductive substance. The discharge printing by means of reduction is slow and laborious. It has a poor repeatability, and it is hazardous to the environment.

The reductive substances infest waste water by increasing the consumption of oxygen therein. The decolourisation process with a reductive substance requires steaming, which should take place accurately at a determined temperature, typically at 102°C, and the aqueous vapour must not condensate in such a manner that drops would fall on the surface of the textile product.

By means of the method according to the invention it is possible to avoid the above-mentioned problems. The method according to the invention is characterized in that colour is removed by means of an oxidizing treatment. The discharging agent according to the invention is characterized in that it comprises at least one oxidizing agent intended for decolourisation.

One advantage of the invention is that the method according to the invention can be easily controlled, and the method produces a patterning of higher quality than methods of prior art. The decolourisation can be conducted at normal room temperature, wherein problems caused in known methods by the high temperature and humidity, do not occur.

The textile product to be patterned contains wool, animal hair, silk or polyamide. In addition to a textile product made solely of one fibre, the textile product may contain a mixture of the above-mentioned fibres, and the mixtures may also contain other fibres than those mentioned above. The amount of dyed fibres that can be contained in the textile product without being affected by the discharging agent, nevertheless producing a patterning of sufficient quality, depends for example on the bond of the fabric or knitted fabric. It is possible that even 50 % by weight of the textile product contains such fibres. In fibrous mixtures for example a wool/polyamide mixture of 95/5 % by weight is advantageous, because both fibres can be dyed with similar dyes, and thus the discharging agent affects both fibres. The wool/polyamide mixture also has good abrasion resistance values.

The colour of the textile product may be a result of dyeing, or it may be the natural colour of the fibre, which is possible for example in the case of wool. The textile product may be dyed in a dye bath either continuously or in a batch process, or it may be printed. In the textile product an area having the shape of a desired pattern is treated with a discharging agent containing an oxidizing agent to remove the colour from said area. Especially for wool it is advantageous to use substances intended for the treatment of hair as a discharging agent, because the wool fibre behaves chemically in a similar manner as the human hair.

Reactive dyes or acid dyes, especially low acid dyes are used for dyeing. The reactive dyes bond with the fibre with covalent bonds and the acid dyes with ionic bonds. From the above-mentioned dyes it is possible to select both dyes which do not react with the discharging agent and dyes which react with the discharging agent.

Preferably, the discharging agent has a thickened composition in such a manner that it can be applied accurately and in a clearly defined area in a desired point on the surface of the textile product. The discharging agent has to be thickened in such a manner that it does not start spreading on the surface of the textile product after it has been applied thereon. The composition may be for example salvelike. The discharging agent can be applied on the textile product by methods known as such, for example by brushing with a brush, by using fabric printing methods, or by extruding discharging agent on the fabric.

The discharging agent is applied on a dyed textile product at the point of location of a desired pattern, and it is allowed to work at room temperature for a suitable period of time, a few hours at the most. The effect of the discharging agent can be accelerated by increasing the temperature in which the discharging agent is allowed to affect the textile product. The discharging agent may be supplemented with a dye which does not react with the discharging agent, and which dyes the point of location of the pattern at the same time when dye which reacts with the discharging agent is removed therefrom. The dye which reacts with the discharging agent can be removed entirely or partly, wherein a particular hue is attained. When the textile product has been treated for a sufficiently long period of time, the discharging agent is rinsed off with water, which is advantageously warm. It is also possible to add a washing agent in the water.

The discharging agent contains oxidizing chemicals, e.g. peroxides, such as hydrogen peroxide or magnesium peroxide, and/or inorganic persalts, such as sodium persulphite, potassium persulphite, ammonium persulphite, sodium perborate or a mixture of these. Each oxidizing chemical has its own advantageous pH range, in which the decolourisation is most efficient and/or the effect damaging the fibres is least significant.

The discharging agent may contain alkaline salts, thickening agent and auxiliary substances. The alkaline salts may be for example sodium carbonate, sodium hydrocarbonate, magnesium carbonate, ammonium carbonate, ammonium hydrocarbonate, sodium silicate, or mixtures of these.

The thickening agent may contain for example acrylic acid polymer, cellulose, alginate, polysaccharide, or a mixture of these. The auxiliary substances can be for example substances protecting the fibre, stabilizing agents, or, in addition to the above-mentioned alkaline salts, substances intended for adjustment of pH. When dye is added in the discharging agent, substances promoting the dissolving of the dye as well as protective substances for preventing the dissolving of the dye molecule before fixing to the fibre may be required as auxiliary substances. In the process, a slightly reductive substance such as glucose may be necessary as an auxiliary substance so that it is possible to attain as clearly defined a pattern as possible, even if the discharging agent spread slightly on the surface of the textile product. A slightly reductive substance does not affect the colour, but it prevents the effect of the discharging agent outside the desired patterning area.

In the following, the invention will be described in more detail by means of an example.

### Example 1.

A woollen cloth is dyed with reactive dyes by using the following dyes:
3.0 % Levafix brillant gelb E-3G
1.0 % Levafix brilland blau E-BRA

As for these dyes, Levafix brillant gelb E-3G does not react with the discharging agent, in other words the colour cannot be removed by discharge printing. Levafix brillant blau E-BRA (blue) is a dye that reacts with the discharging agent.

To produce a desired pattern, an area with the shape of the pattern is treated with a discharging agent, which can be for example a substance intended for decolourisation of hair, such as Colour Touch Wella, Welloxon Wella and Goldwell Oxycur Platin. The discharging agent is mixed with a dye Supramin rot GW (red) 1.5%, which does not react with the discharging agent. The discharging agent is allowed to work at normal room temperature for 0.5 to 6 hours. The dye is fixed when it is dry at 100° C for 5 to 10 minutes. Thereafter the discharging agent is washed off from the surface of the textile product with warm water the temperature of which is approximately 30 to 40° C, or with warm water in which washing agents have been added. The percentages presented in the formulas are percentages by weight of the dried matter mass of the mixture used for treating the textile product.

The result is an orange pattern against a green surface. If red dye is not added to the discharging agent, the result is a yellow pattern against a green background.

### Example 2

Blue upholstery fabric with 95/5 % by weight of a wool/polyamide mixture was treated with a discharging agent made of the following constituents:
670 g water
67 g carboxyl methyl cellulose (CMC)
130 g hydrogen peroxide 15%
133 g ammonium persulphate

CMC was dissolved in cold water and the other substances were added. The discharging agent was applied on the surface of the fabric in the shape of the pattern, and it was allowed to work for 6 hours at room temperature. The evaporation of moisture from the surface of the fabric was prevented. After the period of time during which the discharging agent was allowed to work, the discharging agent was washed off. The result attained was a yellow-brown pattern on blue background.

The above-described facts do not restrict the invention, but the invention may vary within the scope of the claims. In the dyeing of the patterns it is possible to use other dye types than reactive and acid dyes, it is, for example, possible to use pigment dyes or metal complex dyes. The textile product can also be patterned in a continuous manner on the same line, if it is, for example in the form of a continuous fabric. The most important aspect in this invention is the fact that a textile product made at least partly of wool, animal hair, silk or polyamide, can be patterned by using an oxidizing chemical in the discharge printing, wherein the patterning of the textile product can be conducted in a more economical manner which is less hazardous to the environment, when compared to methods of prior art.

## Claims

1. A method for patterning a textile product made at least partly of wool, animal hair, silk or polyamide, by means of discharge printing, in which method colour is removed from a dyed textile product or a textile product of natural colour to attain a desired pattern, **characterized** in that the colour is removed with an oxidizing treatment.

2. The method according to claim 1, **characterized** in that the oxidizing treatment is conducted in such a manner that suitably thickened discharging agent containing oxidizing agent is applied on the surface of a dyed textile product or a textile product of natural colour.

3. The method according to claim 2, **characterized** in that the discharging agent is allowed to work at room temperature for 0.5 to 6 hours.

4. The method according to claim 2, **characterized** in that the discharging agent is supplemented with at least one dye which does not react with the discharging agent.

5. The method according to any of the claims 2 to 4, **characterized** in that the discharging agent is washed off from the textile product with warm water.

6. A discharging agent to be used for patterning a textile product made at least partly of wool, animal hair, silk or polyamide, in such a manner that colour is removed from a dyed textile product or textile product of natural colour to produce a desired pattern, **characterized** in that the discharging agent contains at least one oxidizing agent intended for decolourisation.

7. The discharging agent according to claim 6, **characterized** in that it contains a thickening agent.

8. The discharging agent according to claim 6 or 7, **characterized** in that it contains a substance intended for adjustment of pH.

9. Use of products intended for decolourisation of hair to produce patterns by means of discharge printing on the surface of a textile product made at least partly of wool, animal hair, silk, or polyamide.
